

# UNITED STATES PATENT OFFICE.

DANIEL M. SORENSEN, OF TORONTO, ONTARIO, CANADA, ASSIGNOR TO EDSON L. CANNON, OF CLEVELAND HEIGHTS, OHIO.

## LUBRICATING COMPOUND.

1,414,227.

Specification of Letters Patent. Patented Apr. 25, 1922.

No Drawing.

Application filed July 11, 1921. Serial No. 483,997.

To all whom it may concern:

Be it known that I, DANIEL M. SORENSEN, a subject of the King of Great Britain, residing at Toronto, in the county of York, 5 in the Province of Ontario, Canada, have invented a certain new and useful Lubricating Compound, of which the following is a specification.

In the application of oil for lubricating 10 purposes in machinery and internal combustion engines and particularly in automobiles, it is invariably found that after more or less extended use, and depending on the presence of foreign matters therein and to 15 a large extent also upon the viscosity of the oil, such lubricants gradually deteriorate, the oil globules break down and become gradually inefficient for the purposes of lubrication, and by reason thereof a frequent 20 renewal of the oil is necessary.

Ordinary lubricants also tend to create a glaze upon surfaces which are intentionally brought together for frictional purposes— 25 as, for example, the bringing of a brake band into contact with a brake drum—and render such contact ineffective for the purposes of the contact.

My compound is intended to prevent such deterioration of the oil lubricants as above 30 mentioned and to prevent the formation of the glaze above referred to.

In preparing my compound, I employ as a base or foundation an ordinary neutral lubricating oil (such as defined in Vol. 2 35 of The American Petroleum Industry, by Bacon and Hamor, published by McGraw-Hill Book Company, Inc., at New York in 1916) having a body varying in viscosity from 200° to 300°, Saybolt, at 100° F. To 40 such base I add not more than 10% in quantity of a pure soap produced by saponifying fish, vegetable, or animal, oil with ammonia or other appropriate alkali and heating the soap to liquefy the same 45 and render it miscible with such base. The mixture is then agitated to form a uniform or homogeneous compound and is then passed through an appropriate filter or strainer to eliminate all solid or semi-solid 50 constituents or foreign matter.

The lubricating compound, prepared in

the manner above set forth, does not deteriorate or break down under the influence of heat of ordinary intensity generated by moving surfaces in contact, as do ordinary 55 lubricating oils. It creates and maintains a lubricating film between the frictional surfaces and, in the case of automobile engines, this results in increased mileage per gallon of fuel gasoline. The compound not 60 being injuriously affected and carbonized by heat, the parts to which it is applied will not become carbonized, as is the case where ordinary lubricants are employed. Furthermore, when used upon frictional surfaces 65 which are not continuously in contact, but which are brought together at irregular intervals, my compound does not form a hard glazed deposit thereon, as is the case with ordinary lubricating oils, but creates a soft 70 film or surfacing which acts as a cushion between the two contiguous surfaces and prevents them from slipping.

The process of treating the brake bands to prevent the formation of a glazed deposit 75 forms the subject matter of my copending application No. 546543, filed March 25, 1922.

I claim:

1. A lubricating compound particularly 80 useful for preventing the formation of hard glazed surfaces on friction bands consisting of a base of neutral oil having an ammonia soap mingled therewith.

2. A lubricating compound particularly 85 useful for preventing the formation of hard glazed surfaces on friction bands consisting of a base of mineral oil having a viscosity of from 200° to 300° and having an ammonia soap mingled therewith.

3. A lubricating compound particularly 90 useful for preventing the formation of hard glazed surfaces on friction bands consisting of a base of mineral oil having a viscosity of from 200° to 300° and having mingled therewith not more than ten per 95 cent of an ammonia soap.

DANIEL M. SORENSEN.

Witnesses:

J. J. MACCLENNAN,  
E. CORRIGAN.